

**1**

3,482,963

**METHOD FOR PRODUCTION OF PARTICULATE METAL**

Oliver Osborn, Lake Jackson, Tex., and John C. Robertson, Midland, Mich., assignors to The Dow Chemical Company, Midland, Mich., a corporation of Delaware  
No Drawing. Filed Oct. 17, 1966, Ser. No. 586,944  
Int. Cl. C22c 1/08; B22f 1/00

U.S. CL. 75—.5

10 Claims

**ABSTRACT OF THE DISCLOSURE**

A composite body having a porous matrix structure of crushable, friable material and having solid material contained within the pores of the matrix structure is provided. The composite body is crushed to free particulated metal from the matrix structure, thereby providing a mixture of particulate metal and matrix material which has been reduced to a predetermined degree of fineness.

This invention relates to the preparation of particulate metals, and more particularly to the production of particulate light metals such as magnesium, aluminum and alloys thereof.

Methods well known for the production of particulate metals include, for example, the atomization of molten metal by means of the impingement of a stream of molten metal upon a rapidly rotating disc (Br. 510,320), or by the impingement of a high velocity gas jet upon a thin stream of molten metal (U.S. 2,676,359), by means of shot towers, by the shock chilling of gaseous metals, and by the mechanical reduction of masses of solid metal by machining, ball-milling, and other mechanical means well known in the art.

These art processes suffer from one or more of many disadvantages including: (1) the use of complex and expensive equipment and controls, (2) the hazardous handling of molten or gaseous metal at high temperatures and the attendant corrosion problems involved in such handling, (3) fire and ignition hazards either inherent in the handling of liquid or gaseous metals or resulting from the generation of large quantities of heat in the mechanical reduction of solid metal to a finely divided state, (4) the necessity of accomplishing the desired size reduction and rapidly cooling the finely divided metal while maintaining a carefully controlled inert atmosphere, (5) high energy requirements, and (6) low yields of comminuted metals of the desired particle size.

It is a principal object of the present invention to provide an inexpensive method for the production of particulate metals which is easily carried out with simple equipment. Another object is to provide a method which requires a minimum of energy to reduce masses of solid metal to a finely divided state. A further object is to provide a method wherein fire hazards are minimized, particularly with light metals such as magnesium. Other objects and advantages will become apparent hereinafter.

In carrying out the process of the present invention a composite body having a porous matrix structure of crushable, friable material and having solid metal contained within the pores of the matrix structure is provided. The composite body is crushed to free particulated metal from the matrix structure, thereby providing a mixture of particulate metal and matrix material which has been reduced to a predetermined degree of fineness. The particulate metal may, if desired, be separated and recovered from said mixture by a variety of means well known to one skilled in the art such as, for example, by screening, flotation, cyclone separation and the like.

One unexpected advantage of the present invention is that the present novel process provides for the direct prep-

**2**

aration of useful mixtures of the particulate metal and the matrix material. For example, where the matrix material is a reducible fuel such as coke and the metal is magnesium, the resulting particulate mixtures are suitable for use as components of incendiary bombs, pyrotechnics, and explosives.

The present invention is usually carried out by providing a porous, crushable medium having interconnected pores of predetermined size, said medium being thermally stable and not detrimentally attacked at process temperatures, preheating said porous medium, introducing molten metal into the pores of said preheated porous medium, and cooling the thus impregnated porous medium to solidify the metal within said pores. The cooled composite body is then subjected to sufficient crushing action by employing any suitable means such as, for example, a ball-mill, hammer-mill, crushing rolls, or the like to particulate the solidified metal and to reduce the matrix material to a predetermined degree of fineness. The control of the crushing operation and the selection of the equipment by which it is carried out will depend upon several factors. It is usually desirable to reduce the particulate metal to a particulate size corresponding substantially to the predetermined pore size of the porous medium, i.e., to shear or fracture the metal which was contained within the inner-connecting passages between the pores of the matrix material. The friability of the matrix material, the particle size to which it is to be reduced and like considerations will determine the extent and nature of the crushing operation. If it is desired to separate and recover the particulate metal from the matrix material other factors to be considered or controlled to achieve optimum separation, as will be well understood by one skilled in the art, will include the relative volumes, densities, and average particle sizes of the particulate metal and the matrix material.

In a preferred embodiment, the metal to be particulated is introduced into porous media by vacuum casting, i.e. utilizing said porous media as mold forms. Conventional vacuum casting techniques well known in the art can be employed. For example, the integral porous bodies to be impregnated and a sufficient quantity of the solid metal to be cast are placed in a suitable vessel. The vessel is closed, evacuated, and heated to melt the metal and immerse the porous bodies in molten metal. The vessel is then back-filled with an inert gas to relieve the low pressure and substantially completely impregnate the porous bodies.

However, in a more preferred vacuum casting technique, the integral porous mold bodies of suitable refractory material having interconnected pores of predetermined size, said pores being filled with an atmosphere which reacts with the molten metal to be cast to produce a condensed solid oxidized form of said metal which has a low vapor pressure at the casting temperature, are immersed into the molten metal. Substantially complete filling of said pores with molten metal occurs as a vacuum is produced by the reaction between the gas in the pores of the mold bodies and the metal being cast. When the metal to be cast is magnesium, for example, and the pores of the mold bodies are filled with air, the required vacuum is generated as the molten magnesium reacts with the oxygen and nitrogen of the air to form magnesium oxide and magnesium nitride. When the metal is to be cast is aluminum, the pores of the mold bodies may be filled with oxygen. Following the cooling of the metal impregnated composite bodies to solidify the metal, the cooled composite bodies are ground or crushed to free the metal from the matrix material and usually also to break or shear the metal which was contained within the inner-connecting channels or passages between said pores so as to obtain metal particles of said predetermined size.

mined desired size. The particulate metal is then separated from the residual finely divided matrix material and subsequently recovered as hereinbefore described.

An unexpected advantage of the present method is that it has been found that metal impregnated porous media such as, for example, coke, porous carbon, porous alumina and basic ( $MgO-SiO_2$ ) brick, are quite friable and thus easily reduced by crushing or grinding to a sufficiently reduced size to permit ready separation of very finely divided matrix material from the particulate metal by conventional screening. For example, magnesium impregnated metallurgical coke has been hammer-milled so that substantially complete separation of the resulting mixture of pulverized coke and magnesium metal particles was achieved, the bulk of the coke passing through a U.S. Standard 270 mesh screen and approximately 95 percent of the magnesium metal particles being retained on the 270 mesh screen.

Another advantage of the present method is that the particle size of the particulate metal to be produced can be largely controlled by selection of a porous matrix or carrier material of the desired porosity. Further particle size control can be achieved by proper selection of the type of crushing equipment and conditions employed as is understood by one skilled in the art, and as hereinbefore described.

Carrier materials suitable for use in the present method are those which are inert to the metal at process temperatures, are readily crushable, and have melting points higher than that of the metal. Illustrative commercially available materials are, for example, coke, porous carbon, porous alumina, porous  $MgO-SiO_2$  brick, porous burnt lime and porous zirconia.

Carriers of a desired porosity also can be made expressly for use in the method of the present invention. For example, briquettes of calcined dolomite can be prepared from a briquetted mixture of  $MgO-CaO$ , a carbonaceous fuel and water by removing the water at a temperature of about 500° F., burning out the carbonaceous material at a temperature of from about 1200 to 1800° F., and sintering the briquettes at a temperature of about 2500° F. Metals vacuum cast in such synthetic briquettes will have a particle size and particle size distribution substantially that of the carbonaceous material used in forming the briquettes.

The present process is suitable for preparing a variety of metals in particulate form, and is especially suitable for preparing particulate light metals such as magnesium, aluminum and alloys thereof which are not readily fabricated in finely divided form.

The production, transfer and other handling of molten metal, the grinding or crushing of metal impregnated composites, and subsequent separation and metal recovery operations and the like can be carried out using conventional techniques and equipment as is well understood by one skilled in the art.

The following examples will serve to illustrate further the present invention but are not meant to limit it thereto.

#### EXAMPLE 1

A piece of porous aluminum oxide (alumina) weighing 3.69 grams was preheated in air at about 2000° F. for about one hour. The hot alumina was then immersed into a magnesium melt at about 1400° F. for about one minute. The piece was withdrawn from the melt and quenched by covering with a carbonaceous fire extinguishing powder. When the resulting magnesium impregnated alumina had cooled, the magnesium adhering to the surface of the piece was removed. The composite magnesium impregnated aluminum oxide was then weighed and found to contain 12.14% magnesium by weight. The magnesium-alumina composite was ground manually using mortar and pestle. The alumina matrix crumbled easily. The resulting mixture was screened and

found to contain magnesium particles ranging in size from about 200 microns to about 50 microns.

#### EXAMPLE 2

Following the procedure described in Example 1, a porous carbon matrix having a porosity of about 48%, an apparent average pore diameter of 69 microns, and weighing 10.69 grams was preheated in air at about 2400° F. and immersed into molten magnesium at about 1380° F. The resulting magnesium impregnated carbon contained 32.3% magnesium by weight. Sieve analysis following grinding by mortar and pestle showed the magnesium particles to range in size from about 200 to about 75 microns.

15

#### EXAMPLE 3

Using the procedure of Example 1, a piece of porous carbon having a porosity of 48%, an average pore diameter of 33 microns, and weighing 22.28 grams was preheated at about 2400° F. and immersed into molten magnesium at about 1380° F. The impregnated composite containing 22.9% magnesium by weight was crushed by mortar and pestle. The magnesium particles were found to range in size from about 150 to about 50 microns by screen analysis.

20

25

#### EXAMPLE 4

Using the same procedure, a piece of metallurgical grade coke weighing 17.95 grams was immersed into molten magnesium at about 1410° F. for about one minute after preheating at about 1800° F. The magnesium-coke composite containing about 34% magnesium by weight was crushed by means of mortar and pestle. The average magnesium particle size was estimated to be about 1430 microns by visual observation utilizing a microscope with micrometer eyepiece.

30

35

#### EXAMPLE 5

A piece of commercial basic brick analyzing 71.7%  $MgO$ , 19.8%  $SiO_2$ , 4.5%  $Al_2O_3$ , 1.3%  $CaO$  and 0.7%  $Fe_2O_3$ , having a porosity of 65%, and weighing 10.29 grams was wired into a graphite cup. The cup was inverted and plunged into molten magnesium at about 1390° F. for about one minute with no preheating. The resulting magnesium impregnated brick composite was found to contain 47.2% magnesium by weight. The average size of the magnesium particles was estimated to be about 600 microns by visual observation as in Example 4 after crushing the composite by mortar and pestle.

Various modifications can be made in the process of the present invention without departing from the spirit or scope thereof, it being understood that we limit ourselves only as defined in the appended claims.

We claim:

1. A process for producing particulate metal which comprises:
  - (a) forming an integral composite body comprising a solid, crushable matrix structure, said structure defining a multiplicity of interconnected pores in which a metal is solidified from liquid form within said pores of said matrix structure,
  - (b) crushing said composite body thereby to free particulate metal from said matrix structure and provide a mixture of a particulate metal and particulate metal material.
2. The process of claim 1 and including the step of separating the particulate metal from said mixture of particulate metal and matrix material.
3. A process which comprises the steps of
  - (a) introducing a molten metal into the pores of a solid, crushable matrix structure, said structure being thermally stable at the temperature of said molten metal and not detrimentally attacked by said metal,
  - (b) cooling the metal containing matrix structure to solidify the metal within said structure thereby to provide said integral composite body, and

60

65

70

75

(c) crushing said composite body thereby to free particulate metal from said matrix structure and provide a mixture of a particulate metal and particulate matrix material.

4. The process of claim 3 wherein said molten metal is introduced into said pores of said matrix structure by vacuum casting.

5. The process of claim 4 wherein said metal is selected from the group consisting of magnesium, magnesium-base alloys, aluminum, aluminum-base alloys, and mixtures thereof.

6. The process of claim 4 wherein said porous matrix structure is aluminum oxide (alumina).

7. The process of claim 4 wherein said porous matrix structure is coke.

8. The process of claim 4 wherein said metal is magnesium and said porous matrix structure is coke.

9. The process of claim 4 wherein said matrix structure is porous carbon.

10. The process of claim 4 wherein said metal is magnesium and said matrix structure is porous carbon.

#### References Cited

##### UNITED STATES PATENTS

|           |        |                 |       |        |
|-----------|--------|-----------------|-------|--------|
| 679,901   | 8/1901 | Lovett          | ----- | 241—14 |
| 3,028,330 | 4/1962 | Justheim et al. | ----- | 176—71 |
| 3,072,347 | 1/1963 | Dombrowski      | ----- | 241—29 |

L. DEWAYNE RUTLEDGE, Primary Examiner

T. W. FRYE, Assistant Examiner

U.S. Cl. X.R.

UNITED STATES PATENT OFFICE  
CERTIFICATE OF CORRECTION

Patent No. 3,482,963 Dated December 9, 1970

Inventor(s) Oliver Osborn and John C. Robertson

It is certified that error appears in the above-identified patent and that said Letters Patent are hereby corrected as shown below:

In Col. 4, line 64, delete "metal" and insert --matrix--.

SIGNED AND

SEALED

JUN 23 1970

(SEAL)

Attest:

Edward M. Fletcher, Jr.  
Attesting Officer

WILLIAM E. SCHUYLER,  
Commissioner of Patents